# EUROPEAN PATENT SPECIFICATION

(11) **EP 0 613 740 B1**
(45) Date of publication and mention of the grant of the patent: **10.09.1997**
(21) Application number: 94103041.3
(22) Date of filing: 01.03.1994
(51) Int. Cl.: B21D 24/14

(54) **Process and hydraulic press for the pressing of sheets**
Verfahren und hydraulische Presse zum Pressen von Blechen
Procédé et presse hydraulique pour le pressage de tôles

(30) Priority: 02.03.1993 IT TO930148
(43) Date of publication of application: 07.09.1994
(73) Proprietor: FIAT AUTO S.p.A., 10135 Torino (IT)
(72) Inventor: Da Re', Mario, I-10100 Torino (IT)
(74) Representative: Plebani, Rinaldo

(56) References cited:
- EP-A- 0 438 774
- DE-A- 4 038 866
- GB-A- 1 481 202
- US-A- 4 745 792

## Description

The invention concerns a process for the pressing of metal sheets according to the preamble of claim 1, particularly the deep drawing (drawing) of motor vehicle body components.

The invention also concerns a hydraulic press according to the preamble of claim 5, capable of implementing the above-mentioned pressing process.

In known pressing processes a sheet is installed between a matrix and a punch of the die, clamped with pre-determined force by a blank holder which has the task of restraining the sheet against the matrix in the course of the plastic deformation operation. The value of the clamping pressure exerted by the blank holder against the sheet in the pressing phase is fixed and is determined by trials working initially on a batch of test sheets, to be then kept constant for the entire production phase.

This method of working at "constant pressure" has a number of disadvantages particularly in the case of dies of complex shape and for deep drawing, which generally result in a relatively high percentage of rejects due to the formation of flaws on the sheet or the rupture of the sheet itself.

To overcome these disadvantages EP patent application No. 0348774 by this Applicant proposes using a hydraulic press in which the blank holder is actuated with a clamping pressure that is pulsating or alternately variable with a pre-determined law between a minimum value and a maximum value. However, not even this system has proved to be totally effective in reducing rejects in the pressing of certain particularly complex components or pressing sheets which are made of aluminium or have properties that are different from those of steel sheet. Consequently some steel sheet body components have to be produced with special, very expensive so-called "back-hardening" sheets with a high work-hardening capability; and, however, it is not yet possible to produce vehicles with bodies entirely of aluminium on an industrial scale at acceptable cost unless they are restricted to body shapes that are extremely simple and unacceptable from the style point of view.

The object of the invention is to provide an improved process of the pulsating pressure type disclosed above which enables the disadvantages of the latter to be overcome in a simple and economic manner thus enabling sheets, including aluminium sheets, to be processed in complex shapes at low cost.

This object is achieved according to the invention by a process for the pressing of metal sheets as claimed in claim 1.

In particular, the pulsating pressure variation frequency is between zero and 20 Hz inclusive and is selected at a value that is higher, the lower the hardness of the sheet used. In this way even aluminium sheets become easy to process.

Furthermore, particularly when pressing sheets which require the higher frequencies, such as aluminium sheets, the frequency of the said pulsating pressure is made to vary in the course of the pressing operation, particularly in the course of the active stroke of the punch and in any event so as to obtain at least one pressure variation cycle from zero to the maximum value for every 8-10 mm of depth of drawing of the sheet. In this way the rejects are reduced, substantially to zero, even where very complex pressings are involved.

The process according to the invention can be implemented on a hydraulic press for the pressing of sheets, of the type comprising at least one blank holder controlled by actuators via a hydraulic control circuit comprising valve means for alternately pressurizing/depressurizing the blank holder actuators, as defined in claim 5

Further preferred features and advantages of the process and the press according to the invention will emerge from the detailed description which follows, supplied purely by way of example, with reference to the accompanying drawing, in which :
- Fig. 1 is a schematic perspective view of an embodiment of a press according to the invention; and
- Fig. 2 shows a block diagram of a control circuit for the blank holder of the press in Fig. 1.

With reference to Figs. 1 and 2, in the assembly 1 represents a hydraulic press for the pressing of metal sheets 2, made of steel or aluminium or light alloy, for example, particularly to obtain body components of a vehicle which are known and not shown for reasons of simplicity; press 1 comprises a die 3 formed by least one matrix 4 and at least one punch 5 having a profile that is conjugate and shaped like the body component to be obtained, and a blank holder 6 capable of acting on the sheet 2 in correspondence with a perimetric portion 8 thereof.

According to one of the main features of the invention, the blank holder 6, rather than being made of a single piece, consists of a multiplicity of restraining elements 10, four in number for example, one for each side of the sheet 8, which can be controlled independently of each other. In fact, press 1 comprises a hydraulic circuit 18 to control actuators 20 associated with the blank holder 6, particularly associated, singly or in pairs (or three or more according to need) with each restraining element 10. With reference to Fig. 2 also, the circuit 18 comprises in its turn a valve assembly 22 controlled by an electronic microprocessor unit 23 and capable of controlling the inflow and outflow of control fluid to each actuator 20 associated with each element 10, independently for each said element 10.

In particular, the valve assembly 22 is of the same type as vehicle anti-lock brake systems (ABS) and so is not described for reasons of simplicity. Substantially, it is capable of selectively intercepting the flow supplied by a pump 24 towards each actuator 20 for very short periods of time and, possibly, of connecting the actuator to an outlet 25, so as to generate in the actuators 20 a control pressure variable with a periodic law or with a substantially stepwise profile between zero (corresponding to the point at which assembly 22 completely intercepts the said flow and then prevents it from reaching the actuator 20 and, if necessary, connects the actuator 20 to the outlet 25) and a pre-determined maximum value dependent on the characteristic of the pump 24 and, for example, adjustable via the assembly 22 by drawing under the control of the unit 23 (corresponding to the point at which the assembly 22 connects, directly or with drawing towards a pressure control valve which forms part of that assembly, the actuator 20 with the pump 24).

According to a further preferred feature of the invention the unit 23 is capable of controlling the assembly 22 (for example comprising a set of "on-off" type solenoid valves) so as to be able to vary on a continuous basis the periodicity, i.e. the frequency, of the periodic pressure variation law in the actuators 20, for example between a minimum frequency equal to zero (the pressure does not vary and remains constant) and a maximum frequency equal to approximately 20 Hz. Consequently, each element 10 is capable of applying to the sheet 2 a restraining pressure variable between zero (corresponding to the point at which the actuator/the actuators controlling this element 10 are at zero pressure) and a maximum pressure that is adjustable at will, with a frequency which can also be varied as desired between 0 and 20 Hz.

Finally the control circuit 18 is completed by a hydraulic accumulator 26 for supplying the assembly 22 at constant pressure, a filter 27 and a valve
assembly 28 which controls an actuator 29 (not shown in Fig. 1) for raising the blank holder 6, and also exhaust valves 30 of actuators 20.

Working with the press 1 described it is possible to implement a process of pressing the sheets 2 in which a sheet is drawn between the matrix 4 and the punch 5 in the shape of the component to be obtained, for example, a body component of a motor vehicle, restraining the sheet by means of the blank holder 6 exerting on it a pulsating pressure variable alternately between a minimum value equal to zero and a maximum value which can be pre-determined at will. Following experimental trials conducted by the applicant it has also been found that the pulsating pressure must have a frequency selected according to the mechanical properties of the sheet to be pressed, particularly between zero and 20 Hz inclusive (the installation must be capable of achieving the zero value also, but the minimum operating frequency must be not less than 3 Hz) and of a value that is higher, the lower the hardness/strength of the sheet 2 being processed. For example, if sheet 2 is steel, FePO4 for example (designation according to UNI 5866/77 and EURONORM 130/77) between 0.8 and 1 mm thick the frequency must be relatively low, between 8 and 10 Hz inclusive for example; in contrast, for aluminium sheets 0.7-1 mm thick it is necessary to use higher frequencies, between 14 and 18 Hz inclusive.

In the case of aluminium sheets for deep drawing, however, trials have shown that there continued to be a relatively high percentage of rejects (1 in 5) : this latter problem has been surprisingly resolved according to the invention by causing the frequency of the pulsating pressure to vary in the course of the pressing operation, an operation which the microprocessor 23 can easily be asked to perform by appropriate programming thereof; in practice the restraining pressure on the sheet 2 exerted by the blank holder 6 (or by any component 10 of it) is caused to vary with frequency so as to achieve, in the course of the active stroke of the punch 5 (or in the course of that part of the stroke of the punch 5 in which the sheet 2 is actually in the course of plastic deformation) at least one complete cycle of pressure variation, from zero to the maximum value, for every 8-10 mm of depth of drawing which the sheet 2 undergoes.

Working with the parameters described, a percentage rejects figure practically in the vicinity of zero has been obtained, for both steel and aluminium components. For example, it has been possible to produce the rear door of the "FIAT UNO" vehicle from FePO4 with substantially no rejects whilst at the present time this component is made of a material that is much more expensive and valuable. Similarly, deep-drawn components (depth of drawing of the order of 200 mm) have been produced from sheet aluminium with substantially no rejects by causing the pressure pulsation frequency to vary between zero and the maximum value, between 18 Hz initially and 14 Hz finally. These trials were carried out using a press provided with a blank holder having the following properties :

| | |
|---|---|
| - Working force : | 1000 KN |
| - Maximum working force : | 2000 KN |
| - Working speed : | 25-50 mm/sec |
| - Ascent speed : | 100 mm/sec |
| - Pressure pulsation frequency : | 0-20 Hz |
| - Pressure pulsation amplitude : | 0-1,000 KN |
| - Stroke | 180 mm |
| - Working pressure : | 160 bars |
| - Maximum pressure : | 320 bars |

## Claims

1. Process for the pressing of metal sheets (2) comprising the steps of:
- arranging a sheet (2) between a matrix (4) and a punch (5) of a die which are shaped in the shape of a component to be obtained; and
- deforming the sheet (2) by means of the said matrix (4) and punch (5), restraining the sheet (2) between these latter exerting on the sheet (2), by means of a blank holder (6), a pulsating pressure alternately variable between a minimum value and a maximum value, the said pulsating pressure having a pre-determined frequency;
**characterized** in that said minimum value is equal to zero, said pre-determined frequency being selected according to the mechanical properties of the sheet (2) to be pressed and in such a manner to achieve, in the course of the active stroke of the punch (5), at least one pressure variation cycle from zero to the maximum value for every 8-10 mm of depth of drawing of the sheet (2).

2. Process according to Claim 1, characterized in that the frequency of the said pulsating pressure is between zero and 20 Hz inclusive and is selected at a value that is higher, the lower the hardness of the sheet (2) used.

3. Process according to Claim 1 or 2, characterized in that the frequency of the said pulsating pressure is caused to vary in the course of the pressing operation.

4. Process according to one of the preceding Claims, characterized in that a blank holder (6) is used, sub-divided into a multiplicity of restraining elements (10) which are independent of each other, by means of each of which a pulsating pressure variable with a different law from element to element, between zero and a maximum value, which may differ from element to element, is exerted on the sheet (2) in the pressing phase.

5. Hydraulic press (1) for the pressing of sheets (2), for actuating the process according to anyone of the foregoing Claims, comprising at last one blank holder (6) controlled by actuators (20) via a hydraulic control circuit comprising valve means (22) for alternately pressurizing/depressurizing the actuators (20) of the blank holder (6), wherein said valve means (22) are capable of causing the pressure exerted by the blank holder (6) on the sheet (2) to vary between a pre-determined maximum value and a minimum value equal to zero; the said valve means (22) comprising timing means (23) for selectively varying on a continuous basis the alternate pressurizing/depressurizing frequency of the said actuators (20);
**characterized** in that the blank holder (6) is sub-divided into a multiplicity of restraining elements (10) independent of each other, each provided with at least one independent actuator (20) of its own controlled by the said valve means (22), in order to be able to be pressurized/depressurized with a law different from that of the other actuators (20); said actuators being operated by said valve means (22) and said timing means (23) in such a manner to achieve, in the course of the activity stroke of the punch (5), at least one pressure variation cycle from zero to the maximum value for every 8-10 mm of depth of drawing of the sheet (2).

## Patentansprüche

1. Verfahren zum Umformen eines Metallblechs (2), umfassend folgende Schritte:
- Anordnen eines Bleches (2) zwischen einer Matrix (4) und einem Stempel (5) einer Form, wobei Matrix und Stempel in der Form eines zu erhaltenden Teils geformt sind; und
- Verformen des Bleches (2) mittels der Matrix (4) und des Stempels (5), Rückhalten des Bleches (2) zwischen diesen beiden letzteren, die auf das Blech (2) mittels eines Niederhalters (6) einen pulsierender Druck ausüben, der wechselweise zwischen einem Minimalwert und einem Maximalwert veränderbar ist und eine vorbestimmte Frequenz aufweist;
dadurch **gekennzeichnet,** daß
der Minimalwert gleich Null ist, die vorbestimmte Frequenz gemäß den mechanischen Eigenschaften des umzuformenden Bleches (2) und derart gewählt ist, daß im Verlauf des aktiven Hubs des Stempels (5) zumindest ein Druckveränderungszyklus von Null bis zu dem Maximalwert für jede 8 bis 10 mm Tiefe des Ziehens des Bleches (2) erreicht wird.

2. Verfahren nach Anspruch 1, dadurch gekennzeichnet, daß die Frequenz des pulsierenden Drucks zwischen Null und 20 Hz einschließlich liegt und für sie ein Wert ausgewählt wird, der umso höher ist, je niedriger die Härte des benutzten Bleches (2) ist.

3. Verfahren nach Anspruch 1 oder 2, dadurch gekennzeichnet, daß die Frequenz des pulsierenden Drucks veranlaßt wird, sich während des Umformvorgangs zu verändern.

4. Verfahren nach einem der vorhergehenden Ansprüche, dadurch gekennzeichnet, daß ein Niederhalter (6) benutzt wird, der in eine Vielzahl von Rückhalteelementen (10) unterteilt ist, die unabhängig voneinander sind, wobei mittels jedes einzelnen dieser Elemente ein pulsierender Druck, der nach einer von Element zu Element unterschiedlichen Beziehung veränderbar ist, zwischen Null und einem Maximalwert, der von Element zu Element verschieden sein kann, auf das Blech (2) in der Umformphase ausgeübt wird.

5. Hydraulische Presse (1) zum Umformen von Blechen (2) zum Ausführen des Verfahrens nach einem der vorhergehenden Ansprüche, mit zumindest einem Niederhalter (6), der durch Stelleinrichtungen (20) über einen hydraulischen Steuerkreis gesteuert wird, wobei dieser eine Ventileinrichtung (22) zum wechselweisen Beaufschlagen/Ablassen mit/von Druck der/von den Stelleinrichtungen (20) des Niederhalters (6) umfaßt, wobei der durch den Niederhalter (6) auf das Blech (2) ausgeübte Druck mittels der Ventileinrichtung (22) zwischen einem vorbestimmten Maximalwert und einem Minimalwert gleich Null variierbar ist; wobei die Ventileinrichtung (22) eine Synchronisationseinrichtung (23) zum wahlweise Variieren der wechselweisen Beaufschlagungs-/Ablaßfrequenz der Stelleinrichtungen (20) auf einer kontinierlichen Basis umfaßt;
dadurch **gekennzeichnet,** daß
der Niederhalter (6) in eine Vielzahl von voneinander unabhängigen Rückhalteelementen (10) unterteilt ist, wobei jedes mit zumindest einer eigenen unabhängigen Stelleinrichtung (20) versehen ist, die durch die Ventileinrichtung (22) gesteuert wird, um nach einerm sich von der der anderen Stelleinrichtungen (20) unterscheidenden Beziehung beaufschlagbar/ablaßbar zu sein; wobei die Stelleinrichtungen durch die Ventileinrichtung (22) und die Synchronisationseinrichtung (23) derart betreibbar sind, daß im Verlauf des Aktivhubs des Stempels (5) zumindest ein Druckveränderungszyklus von Null auf den Maximalwert für jede 8 bis 10 mm Tiefe des Ziehens des Bleches (2) erreichbar ist.

## Revendications

1. Procédé d'emboutissage de feuilles métalliques (2) comprenant les étapes de:
mise en place d'une feuille (2) entre une matrice (4) et un poinçon (5) d'un outillage qui sont réalisés en fonction de la forme du composant à obtenir; et
déformation de la feuille (2) au moyen desdits matrice (4) et poinçon (5), tout en retenant la feuille (2) entre ces derniers en exerçant sur la feuille (2), au moyen d'un presse-tôle (6), une pression oscillante pouvant varier de manière alternative entre une valeur minimum et une valeur maximum, ladite pression oscillante présentant une fréquence prédéterminée; caractérisé en ce que ladite valeur minimale est égale à zéro, ladite fréquence prédéterminée étant sélectionnée en fonction des propriétés mécaniques de la feuille (2) à emboutir et de manière à obtenir, pendant la course active du poinçon (5), au moins un cycle de variation de pression entre zéro et la valeur maximale pour chaque tranche de 8 à 10 mm de profondeur d'emboutissage de la feuille (2).

2. Procédé selon la revendication 1, caractérisé en ce que la fréquence de ladite pression oscillante est comprise entre zéro et 20 Hz inclus et est sélectionnée de manière que, plus la dureté de la feuille (2) utilisée est faible, plus la valeur est élevée.

3. Procédé selon la revendication 1 ou 2, caractérisé en ce que la fréquence de ladite pression oscillante est amenée à varier au cours de l'opération d'emboutissage.

4. Procédé selon l'une quelconque des revendications précédentes, caractérisé en ce qu'il est utilisé un presse-tôle (6), sous-divisé en une pluralité d'éléments de retenue (10) qui sont indépendants l'un de l'autre, au moyen de chacun desquels une pression oscillante variable suivant une loi différente d'un élément à un autre élément, entre zéro et une valeur maximum qui peut différer d'un élément à un autre élément, est exercée sur la feuille (2) pendant la phase d'emboutissage.

5. Presse hydraulique (1) d'emboutissage de feuilles (2), destinée à mettre en oeuvre le procédé selon l'une quelconque des revendications précédentes, comprenant au moins un presse-tôle (6) commandé par des actionneurs (20) par l'intermédiaire d'un circuit de commande hydraulique comprenant des moyens formant vanne (22) afin de pressuriser/dépressuriser de manière alternée les actionneurs (20) du presse-tôle (6), dans laquelle lesdits moyens formant vanne (22) permettent de provoquer une variation de la pression exercée par le presse-tôle (6) sur la feuille (2) entre une valeur maximale prédéterminée et une valeur minimale égale à zéro; lesdits moyens formant vanne (22) comprenant des moyens de synchronisation (23) destinés à faire varier de façon sélective en continu la fréquence des pressurisations/dépressurisations alternées desdits actionneurs (20);
caractérisée en ce que le presse-tôle (6) est sous-divisé en une pluralité d'éléments de retenue (10) indépendant l'un de l'autre, chacun comportant au moins un actionneur indépendant (20) de lui-même, commandé par lesdits moyens formant vanne (22), dans le but de pouvoir le pressuriser/dépressuriser suivant une loi différente de celle des autres actionneurs (20); lesdits actionneurs étant commandés par lesdits moyens formant vanne (22) et lesdits moyens de synchronisation (23) de manière à obtenir, pendant la course active du poinçon (5), au moins un cycle de variation de pression entre zéro et la valeur maximale pour chaque tranche de 8 à 10 mm de profondeur d'emboutissage de la feuille (2).
